

Dec. 29, 1931.

T. C. SHEEHAN

1,838,116

METHOD OF MAKING RAZOR BLADES

Filed March 24, 1930

FIG. 1



FIG. 2



FIG. 3



FIG. 4



FIG. 5



FIG. 6



INVENTOR

Thomas C. Sheehan  
BY  
Sydney J. Prescott  
ATTORNEY

## UNITED STATES PATENT OFFICE

THOMAS COMLINS SHEEHAN, OF UPPER MONTCLAIR, NEW JERSEY, ASSIGNOR TO  
DURHAM DUPLEX RAZOR COMPANY, A CORPORATION OF NEW YORK

## METHOD OF MAKING RAZOR BLADES

Application filed March 24, 1930. Serial No. 438,572.

This invention relates to razor blades particularly safety razor blades of the flexible double edged type, and to a method of making the same.

5 The main object of the invention is to produce an improved safety razor blade which is free from certain defects or disadvantages inherent in most blades of this type. One of these disadvantages is that due to the thinness of the ordinary blade of this type the edges are not provided with a backing sufficiently rigid for best results. Accordingly it is a principal object of the invention to provide a blade which is transversely flexible to 10 fit holders whose holding surfaces are transversely curved and at the same time providing an inflexible relatively thick edge section for properly supporting the blade edge.

Another object is to prevent breakage along 20 the mid section of the blade which is weakened by center holes or a longitudinal slot by providing a relatively thick inflexible mid section.

Another object is to provide such a blade in 25 which ample transverse flexibility is attained despite the inflexible mid sections and edge sections by flexible sections connecting the edge section with mid section.

Another principal object of the invention is 30 to provide a method of making razor blades of the above type which will produce cheaper and better razor blades. To this end it is an object of the invention to provide a method for producing thin flexible sections connecting relatively thick inflexible mid and edge 35 sections by rolling and grinding sections of the blade, and by this procedure to produce an improved internal structure to the steel forming the blade.

40 Another object is to provide flexible portions of the blade of sufficient width and of sufficiently uniform thickness to distribute bending stress over a considerable area thus eliminating breakage.

45 With these and other objects not specifically mentioned in view the invention consists in certain constructions and steps which will be hereinafter fully described and specifically set forth in the claims hereunto appended.

50 In the accompanying drawings which form

a part of this specification and in which like characters of reference indicate the same or like parts, Fig. 1 is a front elevation of rolling means for producing razor blades in accordance with the method of the invention; Fig. 55 2 is a sectional side elevation of the rolling means shown in Fig. 1; Fig. 3 is a front elevation partly broken away of means for producing the improved razor blades in accordance with the improved method; Fig. 4 is a front 60 elevation partly broken away of rerolling means for carrying the invention into effect; Fig. 5 is a plan view of a razor blade embodying the invention; Fig. 6 is a sectional view on the line 6—6 of Fig. 5.

65 A razor blade carrying the invention into effect has inflexible edge sections and an inflexible mid section for properly supporting the edge and preventing breakage at the slotted or perforated mid section, together with flexible sections connecting said edge sections with said mid sections so as to provide sufficient flexibility to fit curved holders. Preferably the flexible sections are toughened by 70 rolling and rerolling.

75 The method employed in executing the invention consists in rolling ridges in the steel from which the blade is made grinding off or otherwise removing the tops of the ridges and rerolling the remainder into a symmetrical 80 position with respect to the opposite surface of the steel.

85 Referring to the drawings, a strip of steel stock of suitable thickness, in the present instance of approximately fifteen thousandths of an inch, is heated to the proper temperature and then rolled between a pair of rollers 11 and 12. One of these rollers has a pair of shallow grooves 13 about its periphery and the other has a pair of opposed cooperating 90 shallow ridges 14 extending toward the bottom of the grooves 13. As will be seen from Figs. 1 and 2 grooves 13 and ridges 14 are so related that the material of the strip is offset or struck up from the remainder of the 95 strip along the length thereof to produce shallow ridges 24 in the strip. The height of the ridge 24 is in the present embodiment approximately nine thousandths of an inch.

100 The strip is now preferably cooled and

- then subjected to a grinding operation such as that shown in Fig. 3. In this grinding operation the upper side of the ridges is ground off flush or nearly flush with the remaining surface of the strip by means of 5 grinding wheel 15 acting in opposition to roller 16 having guiding and supporting ridges 17, leaving a pair of thin sections of approximately six thousandths of an inch in 10 thickness, approximately that of the usual thin flexible blade. Next these thin sections, after the strip has been properly reheated, are by the means illustrated in Fig. 4 rolled or struck back into a symmetrical position 15 with respect to the opposite surface of the steel strip. These means consist of a pair of cooperating rollers 18 and 19 each having opposed low ridges 20 and 21 which serve to force the material into the symmetrical position referred to and at the same time insure 20 perfect flatness thereof. The strip thereafter is cut into blades of the shape shown in Fig. 5 and the opposite edges thereof are sharpened to form a blade of the cross section shown, somewhat exaggerated for clearer illustration in Fig. 6, provided with thick inflexible edge sections 22 and a thick inflexible mid section 23 connected by thin flexible sections 24. 25
- 30 It will be noted that the method described is considerably simpler and cheaper than obtaining the same shape by the relatively difficult and intricate process of machining or grinding out two grooves on either side of the material. The blade may also be provided 35 with center holes or an axially extending central slot. Since the thin connecting section is of uniform thickness across its considerable width there is no one point at which 40 the greater part of the bending occurs and the bending effect is accordingly distributed over a considerable area thus reducing the chance of breakage. For this reason and because the thickened edge portions are less 45 subjected to burning, the present blade may be given a higher temper than the usual blade of this type. 50 One advantage of the rolling and rerolling process above stated is that the grain or fiber 55 of the steel, in the strip, is toughened instead of being weakened as would be the case if the material removed were ground or machined away from both sides of the blade. This produces a better blade less liable to breakage 60 and requiring less finishing to attain a smooth 65 polished appearance.
- What is claimed is:—
1. The sequence of steps in a method of making razor blades which consists in rolling 60 ridges in the steel of which the blade is made, grinding off the tops of the ridges, and re-rolling the remainder into a symmetrical position with respect to opposite surfaces of the steel. 65
  2. The method of making razor blades 70
3. The method of making razor blades from steel strip which consists in heating the strip, rolling flat longitudinal ridges in the strip, cooling the strip, grinding off the upper sides of the ridges, reheating the strip and re-rolling the remainder of the ridges into symmetrical position with respect to the opposite surfaces of the strip. 75
- In testimony whereof, I have signed my name to this specification.
- THOMAS COMLINS SHEEHAN.
- 80
- 85
- 90
- 95
- 100
- 105
- 110
- 115
- 120
- 125
- 130